

# UNITED STATES PATENT OFFICE.

ROBERT CHARLES MENZIES AND JOHN EDINGTON AITKEN, OF MUSSELBURGH,  
SCOTLAND.

## MANUFACTURE OF PAPER SUITABLE FOR SECURITY-CHECKS.

1,086,386.

Specification of Letters Patent.

Patented Feb. 10, 1914.

No Drawing.

Application filed January 26, 1912. Serial No. 673,697.

*To all whom it may concern:*

Be it known that we, ROBERT CHARLES MENZIES and JOHN EDINGTON AITKEN, both subjects of the King of the United Kingdom of Great Britain and Ireland, and residing at Musselburgh, Scotland, have invented a certain new and useful Improvement in the Manufacture of Paper Suitable for Security-Checks, of which the following is a specification.

This invention relates to improvements in the art of producing paper suitable for security checks, stamps and other documents, by incorporating in the paper pulp in the process of manufacture of paper, or impregnating the partially or completely manufactured paper with, a compound of such nature that when the paper so treated is written or printed on with ordinary ink a reaction will take place as a result of which the color of the ink will be indelibly mordanted in the fibers of the paper.

According to the invention, there is incorporated in the paper pulp, or the partially or completely manufactured paper is impregnated with, a soluble thiocyanate, preferably thiocyanate of ammonium, and a soluble salt of lead, desirably in such proportions that the insoluble thiocyanate of lead produced by the combination, will amount to 5 to 20 per cent. of the weight of the paper more or less; or there may be added directly to the pulp or paper thiocyanate of lead, desirably in the proportion of

5 to 20 per cent. of the weight of the paper 35 more or less.

Having now described our invention, what we claim and desire to secure by Letters Patent of the United States is:—

1. The herein described improvement in 40 the manufacture of paper for security checks and other documents, which consists in subjecting the paper material to the action of a solution of a thiocyanate and of a solution of salt of lead and producing in the paper, 45 by reaction, thiocyanate of lead.

2. The herein described improvement in 50 the manufacture of paper for security checks and other documents, which consists in subjecting the paper material to the action of a 55 solution of thiocyanate of ammonium and of a solution of a salt of lead, and producing in the paper, by reaction, thiocyanate of lead.

3. Paper loaded with thiocyanate of lead. 55

4. Paper loaded with thiocyanate of lead in about the proportions of not less than 5% and not more than 20% of the weight of the paper.

In testimony whereof we have signed our 60 names to this specification in the presence of two subscribing witnesses.

ROBERT CHARLES MENZIES.  
JOHN EDINGTON AITKEN.

Witnesses:

WILLACE FAIRWEATHER,  
JOHN McCLEARY.